

## UNITED STATES PATENT OFFICE

2,163,781

## PHOTOGRAPHIC DEVELOPING PROCESS

John Eggert, Leipzig, and Bruno Wendt, Dessau, Germany, assignors, by mesne assignments, to Agfa Ansco Corporation, Binghamton, N. Y., a corporation of Delaware

No. Drawing. Application June 1, 1936, Serial No. 82,930. In Germany June 7, 1935

5 Claims. (Cl. 95—88)

Our present invention relates to photographic developers.

One of its objects is to provide a new class of developers. Further objects will be seen from the 5 detailed specification following hereafter.

For photographic development there have been used hitherto compounds which, apart from a few exceptions, belong to the group of aromatic polyhydroxy-compounds or of aromatic 10 aminohydroxy- and amino-compounds.

According to this invention the developer is a compound of an aliphatic or heterocyclic series containing the atomic grouping  $-\text{CO}-\text{CHNH}_2-$  or  $-\text{C}(\text{OH})=\text{CNH}_2-$ , that is to say compounds 15 which contain in adjacent position a CO-group and a  $\text{CHNH}_2-$  group, or in the enol-form an hydroxy- and an amino-group attached respectively to two doubly-linked carbon atoms. Any substituents may take the place of hydrogen 20 atoms of the amino-group, for instance alkyl, aryl or acyl.

This new group of developers comprises both slow developers which are active only in caustic alkaline solution and also rapid developers which 25 act in presence of sulfite alone. A particular advantage of the new developers is that many develop under certain conditions directly in color without addition of a second component.

Aliphatic members of the group are, for example, diethylamino-acetone, which is a feebly 30 active developer, aminoacetic acid ethyl ester, aminobenzoyl-acetic acid ethyl ester, and like bodies. Of the heterocyclic group there may be mentioned in particular the derivatives of 4-aminopyrazolone-(5), the hydrazide of ortho- 35 amino-phthalic acid, 3-amino-4-keto-2-imino-tetrahydrothiophene and 3-amino-4-hydroxy-2-keto-furane-dihydride.

The following examples illustrate the invention:

## Example 1

The following mixture is used to develop gas-light paper in brown tints:

|                              |                                         |       |   |
|------------------------------|-----------------------------------------|-------|---|
| 45                           | $\alpha$ -amino-acetic acid ethyl-ester | grams | 6 |
| Sodium sulfite (anhydrous)   | do                                      | 20    |   |
| Sodium carbonate (anhydrous) | do                                      | 10    |   |
| Potassium bromide            | gram                                    | 0.5   |   |
| Water                        | cc                                      | 1000  |   |

## Example 2

The following mixture is used for rapid and brilliant development of negatives:

|                              |                                          |       |   |
|------------------------------|------------------------------------------|-------|---|
| 55                           | 1-phenyl-3-methyl-4-amino-pyrazolone-(5) | grams | 5 |
| Sodium sulfite (anhydrous)   | do                                       | 20    |   |
| Sodium carbonate (anhydrous) | do                                       | 10    |   |
| Potassium bromide            | gram                                     | 0.5   |   |
| Water                        | cc                                       | 1000  |   |

## Example 3

The following developer yields, besides the silver picture an intensely yellow dyestuff picture, which remains when the silver picture has been dissolved, for example by conversion into silver 5 halide and fixing:

|                                                     |       |      |
|-----------------------------------------------------|-------|------|
| 1-para-chlorophenyl-3-methyl-4-amino-pyrazolone-(5) | grams | 5    |
| Sodium sulfite (anhydrous)                          | do    | 5    |
| Potassium bromide                                   | gram  | 0.5  |
| Water                                               | cc    | 1000 |

What we claim is:

1. A process of developing an exposed silver 15 halide emulsion in a solution of an organic compound having in its molecule a divalent radical corresponding to both the following tautomeric formulae



20

wherein R stands for a radical being a member of the group consisting of hydrogen, alkyl, aryl and acyl radicles.

2. A process of developing an exposed silver 25 halide emulsion in a solution of an aliphatic compound having in its molecule a divalent radical corresponding to both the following tautomeric formulae



30

wherein R stands for a radical being a member of the class consisting of hydrogen, alkyl, aryl and acyl radicles.

3. A process of developing an exposed silver 35 halide emulsion in a solution of a heterocyclic compound having in its molecule a divalent radical corresponding to both the following tautomeric formulae



40

wherein R stands for a radical being a member of the group consisting of hydrogen, alkyl, aryl and acyl radicles.

4. A process of developing an exposed silver 45 halide emulsion in a solution of  $\alpha$ -amino-aceto-acetic acid ester.

5. A process of developing an exposed silver halide emulsion in a solution of 1-p-chlorphenyl-3-methyl-4-amino-pyrazolone-(5).

JOHN EGGERT.  
BRUNO WENDT.

55